

## UNITED STATES PATENT OFFICE

2,233,954

## MAGNESIUM BASE ALLOY

John C. McDonald, Midland, Mich., assignor to  
The Dow Chemical Company, Midland, Mich., a  
corporation of Michigan

No Drawing. Application March 30, 1940,  
Serial No. 327,034

3 Claims. (Cl. 75—168)

This invention relates to magnesium base alloys and more particularly concerns an alloy of this nature having an excellent degree of formability associated with other desirable physical properties such as high tensile and yield strengths.

Magnesium alloys are being widely used in the various structural and mechanical arts where a light weight metal is highly desirable, such as for use in making castings, forgings, and the like. However, the use of these alloys in the rolled form to make sheet metal articles requiring forming operations, such as bending, drawing and the like, has not progressed as rapidly due to the fact that in general alloys of good formability permitting relatively sharp bends to be made without the articles developing external cracks usually have inferior strength characteristics.

It is accordingly the principal object of the invention to provide a magnesium base alloy which can be made into rolled sheet or the like possessing a sufficient degree of ductility or formability to be sharply bent, drawn, or otherwise shaped while having good tensile and yield strengths.

Other objects and advantages will be apparent as the description of the invention proceeds.

My invention resides in the discovery that a

is obtained when the alloy contains from 1 to 5 per cent of zinc, from 2 to 8 per cent of thallium, and from 0.05 to 0.4 per cent of calcium. The specific proportion of each alloying metal and the total amount of the alloying metals to be added depends upon the use for which the alloy is intended. For example, where excellent ductility or formability associated with good yield and tensile strengths is of principal importance, the alloy should preferably contain from 0.5 to 10 5 per cent of zinc, 2 to 7 per cent of thallium, and from 0.05 to 0.4 per cent of calcium. However, in those instances where exceptionally high yield and tensile strengths are more important than formability characteristics the alloy may 10 contain increased amounts of thallium and zinc.

The following table lists some of the properties of rolled sheet metal made from my new quaternary alloy and compares these properties with those of rolled sheet made from related 20 ternary alloys. A comparison of the properties listed illustrates the improvement in the formability and strength characteristics of the new alloy over that of the closely related ternary alloys. In the table the per cent elongation is to be regarded as a measure of the ductility or formability of the specimen.

Table

| 30 | Nominal composition in percent<br>(magnesium—remainder) |      |     | Annealed                          |                                     |                                   | Cold rolled                       |                                     | 30 |
|----|---------------------------------------------------------|------|-----|-----------------------------------|-------------------------------------|-----------------------------------|-----------------------------------|-------------------------------------|----|
|    | Zn                                                      | Tl   | Ca  | Yield strength<br>in lbs./sq. in. | Tensile strength<br>in lbs./sq. in. | Percent elongation<br>in 2 inches | Yield strength<br>in lbs./sq. in. | Tensile strength<br>in lbs./sq. in. |    |
| 35 | 5.2                                                     | 0.2  | —   | 21,000                            | 35,000                              | 15                                | 31,000                            | 37,000                              | 35 |
|    | 1.0                                                     | 5.2  | —   | 19,000                            | 34,000                              | 17                                | 34,000                            | 41,000                              |    |
| 40 | 1.0                                                     | 5.2  | 0.2 | 23,000                            | 35,000                              | 19                                | 39,000                            | 45,000                              | 40 |
|    | 5.1                                                     | —    | 0.2 | 21,000                            | 35,000                              | 15                                | 31,000                            | 37,000                              |    |
|    | 2.9                                                     | 5.3  | —   | 24,000                            | 37,000                              | 14                                | 38,000                            | 44,000                              |    |
|    | 2.8                                                     | 5.1  | 0.2 | 30,000                            | 42,000                              | 14                                | 44,000                            | 48,000                              |    |
|    | 10.1                                                    | —    | 0.2 | 19,000                            | 34,000                              | 16                                | 30,600                            | 36,000                              |    |
|    | 0.9                                                     | 10.2 | —   | 16,000                            | 33,000                              | 15                                | 34,000                            | 42,000                              |    |
|    | 0.9                                                     | 10.1 | 0.2 | 20,000                            | 35,000                              | 17                                | 36,000                            | 43,000                              |    |

45 magnesium base alloy composed of from 0.3 to 8 per cent of zinc, from 1 to 20 per cent of thallium, and from 0.01 to 1 per cent of calcium, the balance being substantially all magnesium, is endowed with the afore-mentioned properties. While the properties of excellent formability or ductility associated with high tensile and yield strengths are manifest over the entire range of the composition indicated, I have found that in 50 general the preferred combination of properties

45 The properties listed in the above table under the section headed by the term "annealed" were obtained by first rolling the alloys at a temperature of from 400° to 550° F. and thereafter annealing them at various temperatures, in the 50 temperature range from 400° to 800° F. The properties selected for the table were those of the annealed specimens which exhibited the maximum elongation. Properties listed in the above table under the section "cold rolled" were ob- 55

tained by subjecting specimens of the alloy which had been hot rolled at a temperature of from 400° to 550° F. to additional rolling in the cold state in order to improve their strength characteristics. The properties selected for the table were those of the cold rolled specimens which showed the greatest tensile and yield strengths while having at least 1 per cent elongation in 2 inches.

10 By comparison of the properties listed in the above table, it will be observed that the combined properties of my new quaternary alloy are superior to those of closely related ternary alloys having similar percentages of alloying ingredients. For example, it will be noted that the alloys containing the lower percentages of alloying ingredients have an exceptionally high elongation or formability coupled with superior strength characteristics in both the annealed and cold rolled state. In the higher percentages of alloying ingredients the formability or ductility is fairly good, while the strength characteristics show an exceptionally high degree of improvement. Similar improvement will be noted throughout the range of alloying ingredients indicated.

20 While the new alloy is most useful in the wrought form, such as sheets, due to its formability characteristics, it may also be suitably used 30 in making castings, forgings, extruded forms and the like. It is further pointed out that my new

alloy is amenable to solution and precipitation heat treatments, which, accordingly, modify its properties.

The new alloy may be compounded in any of the ways known in the art, such as by adding the 5 alloying ingredients to molten magnesium maintained under a suitable flux. The flux should be substantially free from magnesium chloride if the calcium content is to be above about 0.3 per 10 cent. In those instances where the calcium content is to be less than 0.3 per cent, magnesium chloride may be present in the flux without exerting any deleterious effects, but in this case it is preferable to add the calcium last without too 15 much stirring or agitation in order to guard against loss of some of the calcium into the flux.

I claim:

1. A magnesium base alloy containing from 0.3 to 8 per cent of zinc, from 1 to 20 per cent of 20 thallium, and from 0.01 to 1 per cent of calcium, the balance being magnesium.
2. A magnesium base alloy containing from 0.5 to 1.5 per cent of zinc, from 3 to 7 per cent thallium, and from 0.05 to 0.4 per cent of calcium, the 25 balance being magnesium.
3. A magnesium base alloy containing from 4 to 6 per cent of zinc, from 3 to 7 per cent of thallium, and from 0.05 to 0.4 per cent of calcium, the balance being magnesium.

JOHN C. McDONALD.